

1

2,711,395

## CUTTING OIL COMPOSITION

Amos Dorinson, Park Forest, Ill., assignor to Sinclair Refining Company, New York, N. Y., a corporation of Maine

No Drawing. Application November 25, 1953,  
Serial No. 394,499

4 Claims. (Cl. 252—33.4)

My invention relates to cutting oil compositions containing sulfur-chlorinated pinene type additives and particularly to the use of basic barium mahogany petroleum sulfonate to inhibit corrosion caused by and formation of turbidity in such cutting oil compositions.

Mineral oil compositions containing sulfur-chlorinated pinene type additives, for example, sulfur-chlorinated alpha-pinene, are widely used as cutting oils in metal-working processes. It has been found that oil solutions of such additives up to a concentration of about 2 per cent will not stain copper and such solutions are used as cutting oils for copper and copper alloys as well as for ferrous metals. In the working of ferrous metals with such compositions, however, it is often observed that the workpiece acquires a brown stain and that the slideways and other exposed parts of the machine become similarly stained. Furthermore, when solutions of these additives in petroleum oils, especially in solvent-refined oils, stand for a period of time, they become turbid, giving the solutions and undesirable appearance.

I have found that the staining of ferrous metals caused by the corrosive action of cutting oil compositions containing sulfur-chlorinated pinene type additives and the occurrence of turbidity in such compositions can be inhibited effectively or even suppressed entirely by the addition of basic barium mahogany petroleum sulfonate to the composition. Moreover, I have found that basic barium mahogany sulfonate surprisingly is superior to other oil-soluble mahogany sulfonate soaps such as sodium, neutral barium or basic calcium soaps when compared either on the basis of the total sulfonate content or, for the basic soaps, on the basis of reserve alkalinity. The basic barium sulfonate is effective at lower concentrations and for longer periods of time than sodium, neutral barium or calcium sulfonate. Surprisingly, the advantages of basic barium sulfonate are peculiar to it and do not reside separately in either the barium sulfonate or the basicity of the excess alkaline earth hydroxide. Thus, my invention provides advantageous cutting oil compositions containing sulfur-chlorinated pinene type additives which are substantially non-corrosive to ferrous metals and which remain substantially clear on standing.

By a basic barium mahogany petroleum sulfonate, I mean a barium sulfonate derived from the oil-soluble or mahogany petroleum acids obtained by sulfuric acid, oleum or sulfur trioxide treatment of petroleum oils and containing barium hydroxide in excess of that required for neutralization of the acids. The basic barium mahogany sulfonate advantageously is prepared by treating a petroleum oil with oleum or sulfur trioxide, separating the sludge and neutralizing the oil-soluble mahogany acids, i. e. the acid oil, with ammonia, concentrating the resulting ammonium sulfonate by isopropyl alcohol treatment and converting the ammonium sulfonate to basic barium sulfonate by treatment with excess barium hydroxide. Alternatively, the basic barium sulfonate may be prepared by directly neutralizing a sludge-free acid oil with excess barium hydroxide.

2

By a sulfur-chlorinated pinene type additive, I mean a sulfur-chlorinated pinene or mixtures of pinene and fatty compounds such as fatty esters or fatty acids. For example, suitable additives include sulfur-chlorinated, e. g. with sulfur monochloride, alpha-pinene, sulfur-chlorinated mixtures of alpha-pinene and oleic acid or sulfur-chlorinated alpha-pinene and methyl esters of lard oil fatty acids.

According to my invention, I add basic barium mahogany sulfonate to a cutting oil composition containing a sulfur-chlorinated pinene type additive in an amount sufficient to inhibit the corrosiveness and turbidity of the composition. Generally, about 0.03 to 0.6 weight per cent of basic barium sulfonate based on the composition is sufficient and at least about 0.06 per cent is preferred. Larger amounts of sulfonate may be used but economic considerations will generally preclude the use of more than about 0.6 per cent of the basic barium sulfonate. The sulfonate is conveniently added in the form of a preparation containing various concentrations of the active ingredient. For example, about 0.05 to 1.0 per cent of a 60 per cent basic barium sulfonate concentrated preparation or about 0.2 to 4.0 per cent of a 15 per cent dilute preparation is added to the composition. The resulting composition is substantially non-corrosive to ferrous metals and can be used in metal-working processes without undesirable staining of the metal piece being worked or the metal parts of the working machine. Moreover, the formation of turbidity in such compositions is substantially inhibited and a desirable appearance is kept even when the composition stands for long periods of time.

My invention will be further illustrated by reference to the following examples.

### Example I

The corrosiveness of mineral oil compositions containing a sulfur-chlorinated mixture of alpha pinene and methyl esters of lard oil fatty acids additive including such compositions containing basic barium sulfonate or sodium sulfonate was evaluated.

The tests were carried out on mild steel panels (AISI 1018) which were surface ground on both sides, polished with steel wool and washed with pentane just before immersion in the test oil in a container. About half of the panel was kept immersed in the oil during the test. When the panel was first put into the oil, the container was shaken so that the exposed surfaces of the panel were thoroughly wet with the test oil. Thus each test can be used to evaluate the effects of prolonged immersion, of wetting and subsequent exposure to air and finally of reaction at the surface of the oil.

The action of the sulfonate in inhibiting staining and corrosiveness by the sulfur-chlorinated pinene type additives manifests itself by either completely suppressing or markedly inhibiting initiation of staining of the steel panel by the additive and by retarding the rate of growth of a stained spot on the panel once it has formed. Both of these factors are taken into consideration in rating an inhibitor. With an uninhibited oil containing a sulfur-chlorinated pinene type additive, the onset of staining occurs from 7 to 20 days after immersion of the panel depending on the nature of the base oil, the concentration of the additive, the nature of the additive, and such random and fortuitous factors as microscopic cracks and pits in the test panel. Once a panel has been attacked in the absence of an inhibitor, the growth of the stain is rapid and in a matter of a few days the entire panel is covered with a dense, matte, brown tarnish. The onset of tarnish tends to occur sooner and to progress more rapidly in a solvent-refined Mid-Continent oil than in an acid-treated, naphthenic, Coastal oil.

The basic barium sulfonate preparation used in the tests was prepared by subjecting a solvent-treated Mid-Continent oil, having a viscosity of 200 Saybolt Universal seconds at 100° F. and a viscosity index of 85, to the action of five 25 pound portions of 25 per cent oleum per barrel of oil. After separation of the sludge, the acid oil was blown with air to purge it of sulfur dioxide and neutralized with ammonia. The resulting ammonium sulfonate was concentrated by treatment with isopropanol and the concentrated ammonium sulfonate was converted to basic barium sulfonate by treatment with an excess of barium hydroxide. The preparation contained 62.1 per cent basic barium sulfonate, comprising 53 per cent barium sulfonate and 9.1 per cent barium hydroxide. The sodium sulfonate preparation was "Petronate," a commercially available sodium petroleum sulfonate containing about 60 per cent sodium sulfonate. The per cent inhibitor, i. e. basic barium or sodium sulfonate, used in the tests in this example and in the following examples refers to the weight per cent of gross preparation, not the net concentration of the active ingredient therein.

The sulfur-chlorinated pinene type additive was a sulfur-chlorinated mixture of alpha-pinene and methyl esters of lard oil fatty acids which contained 38 to 41 per cent alpha-pinene, 38 to 41 per cent methyl esters of lard oil fatty acids, 9 to 12 per cent sulfur and 9 to 12 per cent chlorine.

When 2 per cent of the sulfur-chlorinated additive in a solvent-refined Mid-Continent oil and no inhibitor was used in the test, the steel panel first showed a stain at 15 days and a strong stain after 60 days. When basic barium sulfonate was added to the above composition in concentrations of 0.1, 0.2 and 0.5 per cent, no stains appeared and the steel panel remained clean and bright after 60 days. With the same oil containing 1 per cent of the additive and no inhibitor, the steel panel first showed a stain at 15 days and a strong stain after 60 days. When basic barium sulfonate was added to the above composition in concentrations of 0.1, 0.2 and 0.5 per cent, no stains appeared and the steel panel remained clean and bright after 60 days.

When a composition of an acid-treated Coastal oil and 2 per cent of the sulfur-chlorinated additive and no inhibitor was used, the steel panel first showed a stain at 21 days and a strong stain after 60 days. When basic barium sulfonate was added to the above composition in a concentration of 0.05 per cent, a stain did not appear on the steel panel for 56 days and only scattered patches were observed after 60 days, and with concentrations of 0.1 and 0.2 per cent, no stains appeared and the steel panel remained clean and bright after 60 days. With the same oil containing 1 per cent of the additive and no inhibitor, the steel panel first showed a stain at 31 days and a strong stain after 60 days. When basic barium sulfonate was added to the above composition in concentrations of 0.05, 0.1 and 0.2 per cent, no stain appeared and the steel panel remained clean and bright after 60 days.

On the other hand, the solvent-refined Mid-Continent oil containing 2 per cent of the sulfur-chlorinated additive and sodium sulfonate in a concentration of 0.05 per cent first showed a stain after 15 days, in 0.1 per cent after 17 days, in 0.2 per cent after 24 days, in 0.5 per cent after 31 days and in 1 per cent after 41 days. A strong stain was present on the panel after 60 days at all these concentrations. When a 1 per cent concentration of the additive was used and 0.05 per cent sodium sulfonate, a stain appeared after 52 days and was fairly strong after 60 days, at 0.1 per cent concentration a weak stain appeared after 60 days, at 0.2 per cent concentration the panel was clean and bright after 60 days, at 0.5 per cent concentration the panel stained at 52 days and had stained patches after 60 days and at 1 per cent concentration the panel was clean and bright after 60 days.

The results clearly indicate that whether the base oil is a solvent-refined Mid-Continent or an acid-treated

Coastal oil and whether the sulfur-chlorinated pinene type additive is present at a 2 per cent or 1 per cent concentration, at concentrations of 0.1 per cent the basic barium sulfonate preparation is an effective inhibitor of staining while at the same concentration, the sodium sulfonate preparation is not effective. Moreover, there is an indication that the basic barium sulfonate can be effective at concentrations as low as 0.05 per cent. Comparison of the two preparations on an equimolar basis, each weight per cent of basic barium sulfonate being equivalent to 0.77 per cent sodium sulfonate, shows the superiority of the basic barium sulfonate in an even more pronounced manner.

#### Example II

The corrosiveness of mineral oil compositions containing a sulfur-chlorinated alpha-pinene additive including such compositions containing the basic barium sulfonate of Example I was also evaluated according to the procedure of Example I. The additive contained 64 to 70 per cent alpha-pinene, 15 to 18 per cent sulfur and 15 to 18 per cent chlorine.

When a mineral oil composition containing the additive in a concentration of 1.08 per cent and no inhibitor was used in the test, the steel panel first showed a stain after 13 days and was lightly stained after 30 days. When basic barium sulfonate in a concentration of 0.1 per cent was added to the above composition, a stain appeared on the steel panel after 13 days but no more than a few stained patches were observed after 30 days. With a concentration of 0.54 per cent of the additive and no inhibitor, a stain appeared after 13 days and the steel panel was sparsely stained after 30 days. When basic barium sulfonate was added to the composition in a concentration of 0.1 per cent, a stain appeared after 13 days but only a few stained patches were observed after 30 days.

The results indicate that the onset of staining by sulfur-chlorinated alpha-pinene is not retarded but further growth of the stain is definitely slowed down.

#### Example III

The corrosiveness of mineral oil compositions containing a sulfur-chlorinated mixture of alpha-pinene and oleic acid additive including such compositions containing the basic barium sulfonate of Example I was evaluated according to the procedure of Example I. The additive contained 38 to 41 per cent alpha-pinene, 38 to 41 per cent oleic acid, 9 to 12 per cent sulfur and 9 to 12 per cent chlorine.

When a mineral oil composition containing the additive in a concentration of 2 per cent and no inhibitor was used in the test, the steel panel showed a stain after 13 days and a strong stain after 30 days. When basic barium sulfonate was added to the above composition in a concentration of 0.1 per cent, the steel panel was dull but not stained after 30 days. With the additive in a concentration of 1 per cent and no inhibitor, a strong stain was observed after 30 days. When basic barium sulfonate was added to the above composition in a concentration of 0.1 per cent, the steel panel was clean and bright after 30 days.

The results show that compositions containing sulfur-chlorinated mixtures of alpha-pinene and oleic acid can be rendered entirely non-staining by the addition of 0.1 per cent basic barium sulfonate.

#### Example IV

The corrosiveness of mineral oil compositions containing the sulfur-chlorinated mixture of alpha-pinene and methyl esters of lard oil fatty acids additive of Example I including such compositions containing neutral barium sulfonates and basic calcium sulfonates was evaluated according to the procedure of Example I.

The neutral barium sulfonate was prepared by treating a basic barium sulfonate with enough acid oil to neutralize

the excess basicity. The basic barium sulfonate was prepared by treating a raw Mid-Continent oil of 200 Saybolt Universal seconds viscosity at 100° F. with oleum in the manner described in Example I. The sludge-free and blown acid oil was neutralized directly with excess barium hydroxide to produce a preparation having a base number of 12 mgms. of KOH per gram and containing 15.8 per cent basic barium sulfonate. On treatment with enough acid oil to neutralize the excess basicity, the resulting neutral barium petroleum sulfonate contained 1.76 per cent barium and 12.2 per cent barium sulfonate.

The basic calcium sulfonate was prepared in the same manner as the basic barium sulfonate described above except that neutralization was carried out with calcium hydroxide. The preparation contained 23.1 per cent basic calcium sulfonate, comprising 22.6 per cent calcium sulfonate and 0.53 per cent calcium hydroxide.

When a mineral oil composition containing 2 per cent of the additive and no inhibitor was used in the test, the metal panel showed a stain after 15 days and a strong stain after 30 days. When 0.83 per cent of neutral barium sulfonate was added to the composition, a stain appeared after 7 days and a moderately strong stain was observed after 30 days while at a concentration of 2.06 per cent, a stain appeared after 12 days and was moderately strong after 30 days. With a concentration of 1 per cent of the additive and no inhibitor, a stain appeared after 15 days and strong stain was observed after 30 days. When neutral barium sulfonate was added to the composition in a concentration of 0.83 per cent, a stain appeared after 7 days and a very light stain was observed after 30 days while at a concentration of 2.06 per cent, a stain appeared after 12 days and stained patches were observed after 30 days.

When compositions containing 2 per cent of the additive and basic calcium sulfonate in a concentration of 0.21 per cent were used in the test, a stain appeared after 7 days and a light stain was observed after 30 days while a concentration of 1.13 produced a stain at 12 days, and stained patches were observed after 30 days. With an additive concentration of 1 per cent and basic calcium sulfonate at a concentration of 0.21 per cent, a stain appeared after 12 days and a light stain was observed after 30 days while at a concentration of 1.13 per cent, a stain appeared after 19 days, and sparse stained patches were observed after 30 days.

The results show that the peculiar advantages demonstrated in Examples I, II and III and in this example of basic barium sulfonate as an inhibitor of the corrosiveness of oil compositions containing sulfur-chlorinated pinene type additives do not reside separately either in the barium sulfonate or the basicity of the excess alkaline earth hydroxide. At a concentration of 0.83 per cent of gross preparation the neutral barium sulfonate furnishes the same concentration of barium as 0.1 per cent of the basic barium sulfonate preparation of Example I and twice the sulfonate concentration and 2.06 per cent of the neutral barium sulfonate is equivalent in sulfonate concentration to 0.5 per cent of the basic barium sulfonate preparation of Example I. However, as shown in the above results, even at a gross concentration of 2.06 per cent neutral barium sulfonate is a poorer inhibitor than 0.1 per cent basic barium sulfonate. Basic calcium sulfonate was used at a concentration of 1.13 per cent which is equivalent to 0.1 per cent of the basic barium sulfonate preparation of Example I in basicity, and at a concentration of 0.21 per cent, equivalent in calcium sulfonate to the barium sulfonate of the basic barium sulfonate at 0.1 per cent concentration. Here too, the basic barium sulfonate is the better inhibitor. In Example I, panels in contact with additive-containing oil inhibited by only 0.1 per cent gross concentration of basic barium sulfonate were clean and bright at the end of 60 days, whereas in these tests neither the

neutral barium sulfonate nor the basic calcium sulfonate were able to keep panels free from stain for as long as 30 days.

*Example V*

Tests were made to determine the effect of basic barium sulfonates on turbidity of mineral oil compositions containing sulfur-chlorinated pinene type additives.

In the tests, basic barium sulfonate in various concentrations was added to mineral oil compositions containing various amounts of sulfur-chlorinated type additives. The oil solutions were allowed to stand for various lengths of time and then were shaken vigorously to disperse the suspended matter uniformly. The turbidity of each solution was measured with a Hellige turbidimeter. The light scattered by the solution of maximum turbidity in each group was taken as 100 per cent and the other solutions were evaluated by comparison; the less the scattering, the less the turbidity.

The basic barium sulfonate inhibitor was that of Example I. The sulfur-chlorinated pinene type additive A was that of Example I and additive B was that of Example II. The results are tabulated below.

|    |                            | Sulfonate Inhibitor, Percent |     |     |     | Standing Time, Days |
|----|----------------------------|------------------------------|-----|-----|-----|---------------------|
|    |                            | 0                            | 0.1 | 0.2 | 0.5 |                     |
| 25 | 2% Additive A: % Turbidity | 100                          | 47  | 8   | 8   | 90                  |
| 30 | 1% Additive A: % Turbidity | 21                           | 8   | —   | 8   | 90                  |
| 30 | 1% Additive B: % Turbidity | 50                           | 11  | —   | —   | 30                  |

The results clearly show the inhibiting effect of basic barium sulfonate on the formation of turbidity in mineral oil compositions containing sulfur-chlorinated pinene type additives.

I claim:

1. Cutting oil compositions of improved corrosion and turbidity inhibiting properties which consist essentially of mineral oil and a sulfur-chlorinated pinene additive to which has been added basic barium mahogany petroleum sulfonate in an amount sufficient to inhibit corrosion and turbidity.
2. Cutting oil compositions of improved corrosion and turbidity inhibiting properties which consist essentially of mineral oil and a sulfur-chlorinated pinene additive, the amount of sulfur-chlorinated pinene additive present being not more than about 2 weight per cent, to which has been added basic barium mahogany petroleum sulfonate in an amount of about 0.03 to 0.6 weight per cent based on the composition.
3. The method of inhibiting the corrosiveness and turbidity of cutting oil compositions which consist essentially of mineral oil and a sulfur-chlorinated pinene additive which comprises adding to the cutting oil composition basic barium mahogany petroleum sulfonate in an amount sufficient to inhibit the corrosiveness and turbidity.
4. The method of inhibiting the corrosiveness and turbidity of cutting oil compositions which consist essentially of mineral oil and a sulfur-chlorinated pinene additive, the amount of sulfur-chlorinated pinene additive being not more than about 2.0 weight per cent, which comprises adding to the cutting oil composition basic barium mahogany petroleum sulfonate in an amount of about 0.03 to 0.6 weight per cent based on the composition.

References Cited in the file of this patent

UNITED STATES PATENTS

- 2,136,391 Miller Nov. 15, 1938  
 2,279,086 Bergstrom Apr. 7, 1942  
 2,493,216 Berger et al. Jan. 3, 1950  
 2,511,250 Fawcett June 13, 1950